# EUROPEAN PATENT SPECIFICATION

(11) **EP 3 767 002 B1**
(45) Date of publication and mention of the grant of the patent: **28.08.2024**
(21) Application number: 19767149.8
(22) Date of filing: 18.01.2019
(51) Int. Cl.: C23C 4/06, B21B 25/00, C23C 4/11, G01N 23/223, C22C 38/00, C22C 38/12, B21B 19/04, C23C 4/123, C23C 4/129, C23C 4/131, C23C 30/00, C22C 38/02, C22C 38/04, C22C 38/08

(54) **PIERCER PLUG**
LOCHDORN
PERCEUR-MANDRINEUR

(30) Priority: 14.03.2018 JP 2018047307
(43) Date of publication of application: 20.01.2021
(73) Proprietor: NIPPON STEEL CORPORATION, Chiyoda-ku Tokyo 100-8071 (JP)
(72) Inventor: HIDAKA, Yasuyoshi, Tokyo 100-8071 (JP); HIGASHIDA, Yasuto, Tokyo 100-8071 (JP); SHIRASAWA, Naoya, Tokyo 100-8071 (JP)
(74) Representative: Zimmermann & Partner Patentanwälte mbB
(86) International application number: PCT/JP2019/001486
(87) International publication number: WO 2019/176279

(56) References cited:
- EP-A1- 2 845 655
- EP-A1- 2 875 876
- EP-B1- 2 896 716
- EP-B1- 3 705 591
- WO-A1-2013/161177
- JP-A- 2001 247 905
- JP-A- 2014 028 395
- JP-A- 2014 028 395
- JP-A- H01 154 808
- JP-A- H03 204 106
- JP-B2- S5 913 924
- JP-B2- S5 913 924
- US-A- 4 393 677
- US-A1- 2010 050 723

## Description

### TECHNICAL FIELD

The present invention relates to a piercer plug.

### BACKGROUND ART

Conventionally, a piercer plug for piercing and rolling to produce a seamless steel pipe is provided with a scale coating on its surface before use to ensure the thermal insulation, lubrication and seizure resistance of the surface.

A scale coating gradually wears down during each round of piercing/rolling. When the scale coating wears out and base material (i.e., plug body) is exposed, the base material may be eroded and/or seize upon the material to be processed. A scale coating significantly wears down during piercing of a material that is difficult to process, such as stainless steel; the coating may wear out just after several passes. Each time this occurs, heat treatment is necessary to form a scale coating once again, which requires several hours to several dozens of hours, meaning poor efficiency.

WO 2009/057471 proposes forming a sprayed coating made from iron and oxides on the surface of the base material of the piercer plug. WO 2014/034376 discloses a piercer plug including a sprayed coating containing iron and iron oxides and, in addition, in mass %, 0.015 to 0.6 % C, 0.05 to 0.5 % Si, 0.1 to 1.0 % Mn, and 0 to 0.3 % Cu.

US 4393677 A discloses a plug for use in a piercing and elongating mill characterizing in that an adherent durable surface layer consisting essentially of iron oxides, i.e. FeO, Fe₃O₄, Fe₂O₃ or mixtures thereof is formed on the surface of the plug by spraying said molten iron oxide powder onto the plug surface to form said layer. The powder may also contain oxides of chromium, nickel, cobalt, copper, manganese and alloys thereof. The plug is preferably coated with a layer of nickel aluminum before the iron oxide powder is sprayed thereon.

Patent document EP2875876-A1 describes a piercer plug with a sprayed coating thereon, wherein the coating comprises Fe, Fe-oxides and Cr. EP2845655-A1 describes a coated piercing plug and a thermal spray method for its manufacture.

### DISCLOSURE OF THE INVENTION

Sprayed coatings have better adhesion with respect to base material and better wear resistance than scale coatings, and can be formed in several minutes to several dozens of minutes. As such, sprayed coatings have longer lives than scale coatings, and, even when a sprayed coating has worn out, it can be restored in a short period of time. Meanwhile, it is desirable to further increase the life of piercer plugs to increase the manufacture efficiency of seamless steel pipes. It is thus desirable to further increase the wear resistance of coatings.

An object of the present invention is to provide a piercer plug with further increased wear resistance.

A piercer plug according to the present invention is as described in the appended claims.

The present invention provides a piercer plug with further increased wear resistance.

### BRIEF DESCRIPTION OF THE DRAWINGS

[FIG. 1] FIG. 1 is a longitudinal cross-sectional view of a piercer plug according to an embodiment of the present invention.
[FIG. 2] FIG. 2 illustrates exemplary equipment used to form a sprayed coating.
[FIG. 3] FIG. 3 is a cross-sectional view of a cored wire.
[FIG. 4] FIG. 4 is a longitudinal cross-sectional view of a piercer plug according to another embodiment of the present invention.
[FIG. 5] FIG. 5 is a longitudinal cross-sectional view of a piercer plug according to yet another embodiment of the present invention.
[FIG. 6] FIG. 6 is a cross-sectional microphotograph of a sprayed coating containing no Cr.
[FIG. 7] FIG. 7 is a cross-sectional microphotograph of a sprayed coating containing Cr.

### EMBODIMENTS FOR CARRYING OUT THE INVENTION

Embodiments of the present invention will now be described in detail with reference to the drawings. The same or corresponding parts in drawings are labeled with the same characters and their description will not be repeated. The size ratios between components shown in drawings do not necessarily indicate the actual size ratios.

### [Construction of Piercer Plug]

FIG. 1 is a longitudinal cross-sectional view of a piercer plug 10 according to an embodiment of the present invention. The piercer plug 10 includes a plug body 11 and a sprayed coating 12.

The plug body 11 is projectile-shaped. Specifically, the plug body 11 has a circular transverse section and is shaped such that its outer diameter increases as it goes from the tip of the plug body 11 toward the rear body's end. The plug body 11 is formed from an iron-based alloy, for example.

The sprayed coating 12 is provided on the surface of the plug body 11. The sprayed coating 12 covers the entire surface of the plug body 11 except for the rear end face of the plug body 11. The thickness of the sprayed coating 12 may not be constant. The sprayed coating 12 is preferably formed such that its portions overlying the tip 11a of the plug body 11 are thicker than those overlying the body's trunk portion 11b.

The sprayed coating 12 contains at least an iron-based alloy and oxides thereof. The sprayed coating 12 may contain other compounds.

The iron-based alloy in the sprayed coating 12 is mainly composed of iron (Fe), and also contains carbon (C), silicon (Si), manganese (Mn) and chromium (Cr), for example. The iron-based alloy in the sprayed coating 12 may contain only one or some of C, Si, Mn and Cr, and may contain elements other than C, Si, Mn and Cr. When viewed microscopically, the chemical composition of the iron-based alloy in the sprayed coating 12 may not be uniform. For example, when viewed microscopically, portions containing almost no Cr and portions with high Cr contents may be present in a mixed manner.

The oxides in the sprayed coating 12 are the oxides resulting from the iron-based alloy being oxidized. Specifically, the oxides in the sprayed coating 12 are iron oxides and complex oxides of iron and chromium, for example. The iron oxides may be FeO or Fe₃O₄, for example. The complex oxides of iron and chromium may be (Fe,Cr)₃O₄, for example. The oxides in the sprayed coating 12 may contain oxides of other metals.

The higher the proportion of metal (i.e., iron-based alloy) that is an ingredient in the sprayed coating 12, the better the adhesion with respect to the plug body 11. On the other hand, the higher the proportion of oxides, the better the heat insulation. The proportion of oxides in the sprayed coating 12 is 25 to 80 vol%, and preferably 35 to 65 vol%. Further, it is preferable that portions of the coating near the plug body 11 have high proportions of metal and portions located toward the surface have higher proportions of oxides. Such a construction will further increase the adhesion with respect to the plug body 11. The volume ratio of oxides can be determined by observing a cross section of the sprayed coating 12 and doing calculations.

In the piercer plug 10 according to the present invention, the chromium concentration determined by analyzing the sprayed coating 12 with X-ray fluorescence analysis (hereinafter referred to as "XRF-Cr concentration") is 3 to 20 mass %.

An XRF-Cr concentration of 3 mass % or higher provides a better wear resistance than a concentration below 3 mass %. This is presumably because the complex oxides of iron and chromium increase the hardness of the sprayed coating 12. On the other hand, an XRF-Cr concentration exceeding 20 mass % results in insufficient lubrication of the sprayed coating 12, which reduces piercing efficiency. The lower limit for XRF-Cr concentration is preferably 5 mass %, and more preferably 8 mass %. The upper limit for XRF-Cr concentration is preferably 18 mass %, and more preferably 16 mass %.

XRF-Cr concentration is measured in the following manner: an X-ray is directed into the sprayed coating 12 through its surface, and the resulting X-ray fluorescence is detected with a detector. The incident X-ray is generated by a 3 mm ø spot collimator with a target of Rh and an output of 40 kV × 100 pA. The detector is a Si drift detector. The concentration of Cr is determined as a mass percentage, where the denominator is the total amount of all the elements detected. The numerator for XRF-Cr concentration includes both the Cr amount in the iron-based alloy and the Cr amount in the oxides.

In the piercer plug 10 according to the present invention, the iron concentration determined by analyzing the sprayed coating 12 with X-ray fluorescence analysis is 50 mass % or higher. The determination of iron concentration by analyzing the coating with X-ray fluorescence analysis involves the same measurement method as for XRF-Cr concentration.

### [Method for Manufacturing Piercer Plug]

An exemplary method for manufacturing the piercer plug 10 will be described below. The method described below is exemplary only, and a method for manufacturing the piercer plug 10 is not limited thereto.

A plug body 11 is prepared. The plug body 11 may be any plug body known to a person skilled in the art.

A sprayed coating 12 is formed on the plug body 11. The sprayed coating 12 may be formed using an arc sprayer 20, shown in FIG. 2.

The arc sprayer 20 includes a spraying gun 21 and a rotating base 24. The spraying gun 21 generates an arc at the tips of a positive-electrode wire 22 and a negative-electrode wire 23 to melt metal, which is then ejected by means of compressed air.

The chemical composition of, and the XRF-Cr concentration in, the sprayed coating 12 may be regulated by adjusting the chemical compositions of the positive- and negative-electrode wires 22 and 23. The positive- and negative electrode wires 22 and 23 may have the same chemical composition or may have different chemical compositions. If wires of different chemical compositions are used, metal from the positive-electrode wire 22 and metal from the negative-electrode wire 23 mix together to form a pseudo-alloy.

Although not limiting, the positive- and negative-electrode wires 22 and 23 may be made of carbon steel or stainless steel, for example. Alternatively, the positive- and negative-electrode wires 22 and 23 may be made of cored wire 30, shown in FIG. 3. The cored wire 30 includes an outer sheath 31 made from carbon steel and a filler 32 filling the outer sheath 31. The chemical composition of the metal ejected from the spraying gun 21 may be changed at will by changing the type of the filler 32.

The longer the distance between the tip of the spraying gun 21 and the surface of the plug body 11 (hereinafter referred to as "spraying distance"), the higher the proportion of oxides in the sprayed coating 12. This is because the oxidation of metal ejected from the tip of the spraying gun 21 progresses along the spraying distance. Although not limiting, the spraying distance may be 100 to 1400 mm, for example. Further, spraying at gradually increasing spraying distances results in higher proportions of metal in portions near the plug body 11 and higher proportions of oxides in portions located toward the surface.

As discussed above, the numerator for XRF-Cr concentration includes both the Cr amount in the iron-based alloy and the Cr amount in the oxides. As such, the XRF-Cr concentration does not significantly change even if the proportion of oxides in the sprayed coating 12 changes. Thus, the XRF-Cr concentration does not significantly change even when the spraying distance is changed.

Spraying is performed while the rotating base 24 rotates the plug body 11 about its axis until the thickness of the sprayed coating 12 reaches a predetermined level. Although not limiting, the thickness of the sprayed coating 12 may be 200 to 3000 pm, for example.

Preferably, the formation of the sprayed coating 12 is followed by heat treatment for diffusion purposes. This achieves higher adhesion between the plug body 11 and sprayed coating 12. For the heat treatment for diffusion purposes, the plug is preferably held at 600 to 1250 °C for 10 minutes or longer, for example. The heat-treatment temperature is more preferably 600 to 1100 °C.

The piercer plug 10 according to an embodiment of the present invention has been described. In the present invention, the XRF-Cr concentration in the sprayed coating 12 is 3 to 20 mass %. This will increase the wear resistance of the piercer plug 10.

The above-described embodiment illustrates an implementation where the plug body 11 is projectile-shaped. However, the plug body 11 may have any shape. For example, the piercer plug may be a plug body 13 with a protruding tip, as shown in FIG. 4, with a sprayed coating 12 formed thereon, or may be a plug body 14 of a divided construction, as shown in FIG. 5, with a sprayed coating 12 formed thereon.

The above-described embodiments illustrate implementations where the sprayed coating 12 is formed by arc spraying. However, a method for forming the sprayed coating 12 is not limited thereto. The sprayed coating 12 may be formed by, for example, plasma spraying, flame spraying, highspeed flame spraying, etc.

### EXAMPLES

The present invention will now be described more specifically by means of examples. The present invention is not limited to these examples.

A model plug mainly composed of 0.15 C, 0.5 Si, 1.0 Ni, 0.5 Mn, 1.5 Mo, 3.0 W, and balance Fe was prepared and a sprayed coating was formed thereon. A positive-electrode wire and a negative-electrode wire were prepared by combining wires of a low-carbon steel, SUS 410 and SUS 430, and cored wires with different Cr concentrations to adjust the compound of the sprayed coating to be formed.

The XRF-Cr concentration in the sprayed coating was analyzed by the method described in connection with the embodiment. The X-ray fluorescence analyzer used was DP-2000 Delta Premium from JEOL Ltd., and the analysis was performed using ALLOY PLUS alloy analysis software from JEOL Ltd.

The Vickers hardness of the sprayed coating of each plug was measured. The Vickers hardness of each plug was obtained by conducting three-point measurement and determining the average of the measurements.

Table 1 shows the relationship between XRF-Cr concentration and average hardness. In Table 1, "-" in the column for XRF-Cr concentration indicates that the XRF-Cr concentration was below the lower limit for analysis.

### [Table 1]

**TABLE 1**

| Mark | XRF-Cr concentration (mass %) | Vickers hardness (Hv) |
|---|---|---|
| A | - | 320 |
| B | 1.04 | 345 |
| C | 3.03 | 380 |
| D | 7.85 | 400 |
| E | 11.52 | 450 |
| F | 15.53 | 500 |
| G | 18.11 | 520 |
| H | 22.30 | 550 |

As shown in Table ,1 the higher the XRF-Cr concentration, the higher the average Vickers hardness.

FIG. 6 shows a cross-sectional microphotograph of the sprayed coating labeled Mark A in Table 1. FIG. 7 shows a cross-sectional microphotograph of the sprayed coating labeled Mark C in Table 1. As illustrated in FIG. 7, a sprayed coating containing Cr was composed of metal and oxides, similar to the sprayed coating containing no Cr (FIG. 6). In these figures, relatively bright portions represent portions made from metal, while dark-gray portions represent portions made from oxides. The ratio between metal and oxides was substantially the same for each of the sprayed coatings prepared for the present application, where the proportion of oxides was about 44 to 55 vol%.

Subsequently, these plugs were used to conduct piercing tests, where the material to be processed was SUS 304, to measure the amount of wear of the coating. Table 2 shows the relationship between XRF-Cr concentration and amount of wear. The column labeled "Ratio of wear to conventional" in Table 2 lists the relative amounts of wear for the sprayed coatings of the plugs, where the amount of wear for the sprayed coating of the plug labeled Mark A represents the value 1.

### [Table 2]

**TABLE 2**

| Mark | XRF-Cr concentration (mass %) | Ratio of wear to conventional | Notes | Remarks |
|---|---|---|---|---|
| A | - | 1 (reference) | - | comp. ex. |
| B | 1.04 | 0.95 | - | comp. ex. |
| C | 3.03 | 0.70 | - | inv. ex. |
| D | 7.85 | 0.70 | - | inv. ex. |
| E | 11.52 | 0.60 | - | inv. ex. |
| F | 15.53 | 0.40 | - | inv. ex. |
| G | 18.11 | 0.50 | - | inv. ex. |
| H | 22.30 | 0.11 | low piercing efficiency | comp. ex. |

As shown in Table 2, the higher the XRF-Cr concentration, the smaller the amount of wear. Particularly, an XRF-Cr concentration of 3 mass % or higher resulted in a reduced amount of wear of up to about 70 % of the level for Mark A. On the other hand, an XRF-Cr concentration exceeding 20 mass % resulted in a reduction in piercing efficiency, making rolling difficult.

These results prove that an XRF-Cr concentration in the range of 3 to 20 mass % increases the wear resistance of a piercer plug.

Although embodiments of the present invention have been described, the above-described embodiments are exemplary only, intended to allow the present invention to be carried out. Accordingly, the present invention is defined by the scope of the appended claims.

## Claims

1. A piercer plug, comprising:
a plug body (11); and
a sprayed coating (12) formed on a surface of the plug body (11),
the sprayed coating (12) containing an iron-based alloy and an oxide of the iron-based alloy,
a chromium concentration determined by analyzing the sprayed coating (12) with X-ray fluorescence analysis being 3 to 20 mass %, wherein
the chromium concentration determined by analyzing the sprayed coating (12) with X-ray fluorescence analysis is measured such that an X-ray is directed into the sprayed coating (12) through its surface, the resulting X-ray fluorescence is detected with a Si drift detector, and the incident X-ray is generated by a 3 mm ø spot collimator with a target of Rh and an output of 40 kV × 100 µA,
the chromium concentration being determined as a mass percentage, where the denominator is a total amount of all elements detected, and the numerator includes both a Cr amount in the iron-based alloy and a Cr amount in the oxides,
wherein a proportion of oxides in the sprayed coating (12) is 25 to 80 vol%, and
wherein an iron concentration determined by analyzing the sprayed coating (12) with X-ray fluorescence analysis is 50 mass % or higher, and wherein
the iron concentration determined by analyzing the sprayed coating (12) with X-ray fluorescence analysis is measured by the same measurement method as for the chromium concentration.

2. The piercer plug according to claim 1, wherein a thickness of the sprayed coating (12) is 200 to 3000 µm.

## Patentansprüche

1. Lochdorn-Stecker, umfassend:
einen Steckerkörper (11); und
eine gesprühte Beschichtung (12), die auf einer Oberfläche des Steckerkörpers (11) ausgebildet ist,
wobei die gesprühte Beschichtung (12) eine Legierung auf Eisenbasis und ein Oxid der Legierung auf Eisenbasis enthält,
eine Chromkonzentration, die durch Analysieren der gesprühten Beschichtung (12) mittels Röntgenfluoreszenzanalyse bestimmt wird, 3 bis 20 Masse-% beträgt, wobei
die durch Analysieren der gesprühten Beschichtung (12) mittels Röntgenfluoreszenzanalyse bestimmte Chromkonzentration so gemessen wird, dass ein Röntgenstrahl in die gesprühte Beschichtung (12) durch ihre Oberfläche hindurch eingestrahlt wird, die resultierende Röntgenfluoreszenz mit einem Si-Driftdetektor detektiert wird, und die einfallende Röntgenstrahlung durch einen 3 mm ø Spotkollimator mit einem Target aus Rh und einer Leistung von 40 kV × 100 µA erzeugt wird, wobei die Chromkonzentration als ein Massenprozentsatz bestimmt wird, wobei der Nenner eine Gesamtmenge aller detektierten Elemente ist, und der Zähler sowohl eine Cr-Menge in der Legierung auf Eisenbasis als auch eine Cr-Menge in den Oxiden aufweist,
wobei ein Anteil der Oxide in der gesprühten Beschichtung (12) 25 bis 80 Vol.-% beträgt, und
wobei eine durch Analysieren der gesprühten Beschichtung (12) mittels Röntgenfluoreszenzanalyse bestimmte Eisenkonzentration 50 Masse-% oder höher ist, und wobei
die Eisenkonzentration, die durch Analysieren der gesprühten Beschichtung (12) mittels Röntgenfluoreszenzanalyse bestimmt wird, durch das gleiche Messverfahren wie für die Chromkonzentration gemessen wird.

2. Lochdorn-Stecker nach Anspruch 1, wobei eine Dicke der gesprühten Beschichtung (12) 200 bis 3000 µm beträgt.

## Revendications

1. Poinçon de dispositif de perçage comprenant :
un corps de poinçon (11) ; et
un revêtement appliqué par pulvérisation (12) formé sur une surface du corps de poinçon (11),
le revêtement appliqué par pulvérisation (12) contenant un alliage à base de fer et un oxyde de l'alliage à base de fer,
une concentration de chrome, déterminée par analyse du revêtement appliqué par pulvérisation (12) au moyen d'une analyse de fluorescence X, de 3 à 20 % en masse,
laquelle concentration de chrome, déterminée par analyse du revêtement appliqué par pulvérisation (12) au moyen d'une analyse de fluorescence X, est mesurée comme suit : un rayon X est dirigé dans le revêtement appliqué par pulvérisation (12) à travers sa surface, la fluorescence X résultante est détectée au moyen d'un détecteur à dérive en Si, et le rayon X incident est généré par un collimateur ponctuel de 3 mm ø avec une cible en Rh et une sortie de 40 kV × 100 µA,
la concentration de chrome étant déterminée en pourcentage en masse, où le dénominateur est la quantité totale de tous les éléments détectés, et le numérateur inclut à la fois la quantité de Cr dans l'alliage à base de fer et la quantité de Cr dans les oxydes,
dans lequel la proportion des oxydes dans le revêtement appliqué par pulvérisation (12) est de 25 à 80 % en volume, et
dans lequel la concentration de fer, déterminée par analyse du revêtement appliqué par pulvérisation (12) au moyen d'une analyse de fluorescence X, est de 50 % ou plus, et
la concentration de fer, déterminée par analyse du revêtement appliqué par pulvérisation (12) au moyen d'une analyse de fluorescence X, est mesurée au moyen du même procédé de mesure que pour la concentration de chrome.

2. Poinçon de dispositif de perçage selon la revendication 1, dans lequel l'épaisseur du revêtement appliqué par pulvérisation (12) est de 200 à 3 000 µm.
